

## UNITED STATES PATENT OFFICE

2,146,040

DEVELOPMENT OF SILVER HALIDE  
EMULSIONS IN COLOR

Gustav Wilmanns, Wolfen kreis Bitterfeld, and  
Wilhelm Schneider, Dessau, Germany, assign-  
ors to Agfa Ansco Corporation, Binghamton,  
N. Y., a corporation of New York

No Drawing. Application April 16, 1936, Serial  
No. 74,816. In Germany April 17, 1935

3 Claims. (Cl. 95—88)

Our present invention relates to development of silver halide emulsions in color.

One of its objects is to provide a process of developing silver halide emulsions in color.

5 Further objects will be seen from the detailed specification following hereafter.

It is known that silver halide layers can be developed in colors. For this purpose there have been used para-aminophenol or dialkyl-10 amino-aniline in admixture with phenol, aniline or such substances as contain a methylene-group capable of reaction. The picture obtained contains silver and the dyestuff, the latter being a quinone-imine dyestuff or an azomethine, accord-15 ing to the nature of the selected components.

Another process consists in using certain poly-20 hydric phenols, such as pyrocatechol or pyrogallol, in an alkaline solution without a sulphite. Both processes suffer from the disadvantage that the solutions have little stability; moreover, the last-named developers give tints which are not very pleasing.

The present invention depends on the obser-25 vation that very beautiful pictures in colors are obtained when an ortho-methyl-aminophenol or a substitution product thereof acts on the silver halide layer in a solution alkaline with alkali carbonate or caustic alkali. After separating the silver, for example with Farmer's reducer, 30 the pure dyestuff picture remains. The developing solutions are remarkably stable. The substituents may be alkyl, such as methyl or ethyl, halogen, alkoxy, such as methoxy or ethoxy, or an amino-group, or a dialkyl amino-group, such as a dimethylamino-group or a diethylamino-35 group. The compounds containing halogen as a substituent have proved to give the best effect.

Suitable ortho-methylaminophenols are, for 40 instance, ortho-methylaminophenol giving a yellow color, 4-chlor-ortho-methylaminophenol giving a brown color, 5-chlor-ortho-methylaminophenol and 4,5-dimethyl-ortho-methylaminophenol giving a yellow color, 4-chlor-6-amino-ortho-methylaminophenol giving a brown color, 45 and 4,6-dimethyl-ortho-methylaminophenol giving a yellow color.

The following examples illustrate the invention:-

Example 1.—A yellow developer is afforded by the following solution:

|                                   |      |     |   |
|-----------------------------------|------|-----|---|
| 4:5-dimethyl-2-methyl-aminophenol | gram | 1   | 5 |
| Sodium hydroxide                  | do   | 0.8 |   |
| Water                             | cc   | 200 |   |

Example 2.—A yellow-red picture is obtained by means of the following developer:

|                     |       |     |    |
|---------------------|-------|-----|----|
| 2-methylaminophenol | gram  | 1   | 10 |
| Potassium carbonate | grams | 10  |    |
| Water               | cc    | 200 |    |

Example 3.—A red picture is obtained by means of the following developer:

|                              |       |     |    |
|------------------------------|-------|-----|----|
| 4-chloro-2-methylaminophenol | grams | 2   | 15 |
| Potassium carbonate          | do    | 15  |    |
| Water                        | cc    | 200 |    |

What we claim is:

1. A process of developing an exposed silver halide emulsion in color, which comprises de-25 positing a dyestuff on the exposed silver halide by treating the exposed silver halide emulsion with a developing solution consisting of an ortho-methylaminophenol, water and an alkali selected from the class consisting of alkali carbonates and caustic alkalies.

2. A process of developing an exposed silver halide emulsion in color, which comprises de-30 positing a dyestuff on the exposed silver halide by treating the exposed silver halide emulsion with a developing solution consisting of water, an alkali selected from the class consisting of alkali carbonates and caustic alkalies, and an 35 ortho-methylaminophenol containing a substituent selected from the class consisting of alkyl, alkoxy, halogen, amino groups and alkyl amino groups, and removing the developed silver from the emulsion.

3. The process as defined in claim 2, wherein the orthomethylaminophenol is 4,5-dimethyl-2-methylaminophenol.

GUSTAV WILMANNS.  
WILHELM SCHNEIDER.